

Oct. 31, 1933

A. T. BERRY

1,932,722

PYROTECHNIC PRODUCT AND METHOD OF MAKING THE SAME

Filed June 9, 1932



Fig. 1.



Fig. 2



Fig. 3.



Fig. 4.

Inventor  
Althea T. Berry  
by Wright Brown Quincy May  
Attest.

## UNITED STATES PATENT OFFICE

1,932,722

PYROTECHNIC PRODUCT AND METHOD OF  
MAKING THE SAME

Althea T. Berry, Wolfeboro, N. H.

Application June 9, 1932. Serial No. 616,198

3 Claims. (Cl. 102—20)

This invention relates to a pyrotechnic product adapted to be applied to a fireplace fire, i. e. fuel burning in an open fireplace, and artificially color the fire.

5 The invention is embodied in an improved product, characterized as hereinafter stated, and in the method of making the same, all as hereinafter described and claimed.

Of the accompanying drawing forming a part 10 of this specification,—

Figure 1 shows in perspective an assembly of elements constituting my improved product, and a box in which said elements are loosely assembled.

15 Figure 2 shows an assembly of said elements united to each other to form a mass adapted to be consumed as a unit.

Figure 3 shows in perspective, and much enlarged, a portion of a shred of commercial excelsior which may constitute the combustible core 20 of an element of the product.

Figure 4 shows the element of Figure 3 in cross section.

The same reference characters indicate the 25 same parts in all of the figures.

In carrying out my invention I assemble a multiplicity of combustible cores *b*, and a semi-fluid adhesive paste, which includes a refractory comminuted ingredient, a glow-emitting flame-coloring ingredient adapted to color a fireplace fire, and an adhesive constituting a binding ingredient. I then agitate the assembly, preferably by placing it in a rotary cement mixer and tumbling until the paste is deposited in the form of 30 coatings *c* on the cores. The coatings are then solidified by drying, preferably by spreading the coated cores on trays and subjecting the coatings to a drying temperature.

Each core and its coating constitutes an element 40 of the improved product.

A suitable quantity of the completed product may be stored loosely in a box *a* having a removable closure (not shown). Relatively small numbers of said elements may be withdrawn from the 45 box and sprinkled more or less extensively on a fire.

Each combustible core *b* may be a shred of excelsior, a planing tool shaving, an auger chip, a strip of wood pulp, or a small piece of any other suitable combustible material adapted to be provided with a coating, as described.

The adhesive constituting the binding ingredient of the paste from which the coatings are formed may be a mixture of ordinary commercial gelatine and water, or liquid or semi-

liquid glue, or a solution of gum arabic. Said adhesive may be otherwise constituted.

The refractory comminuted or powdered ingredient may be magnesium silicate, (talc); or calcium sulphate, (native gypsum); or calcium carbonate. Any other suitable comminuted material or materials may be employed.

The glow-emitting ingredient may include copper chloride and copper sulfate, with or without the salts of other mineral found in sea water, such as sodium, potassium and magnesium, all preferably in powdered or comminuted form.

Any other suitable material or materials, either comminuted, or in solution, may be employed.

In making the paste the ingredients thereof are 70 intimately mixed.

The refractory ingredient and the glow-emitting ingredient are held by the binding ingredient diffused through the coating. The refractory ingredient is not affected by ordinary fireplace 75 heat, and crumbles away while the glow-emitting ingredient, the core and the binding ingredient are being consumed.

When the product is applied to an open fire, the refractory ingredient retards the combustion 80 of the binding ingredient and the glow-emission by the coloring ingredient, and also retards the combustion of the core, so that the flame-coloring effect is more protracted than would be the case if an uncoated combustible core were treated only 85 with a coloring chemical, or if only a comminuted glow-emitting chemical were applied to the fire.

The elements of my improved product may be assembled and adhesively united to each other to form a mass as shown by Figure 2, the mass 90 being of suitable size to be deposited on a relatively small area of a fireplace fire, and consumed as a unit, a protracted localized coloring being the result.

Shredded wood, whose shreds constitute what 95 is known as excelsior, is the best material of which I am aware for the elements hereinbefore called the cores.

My pyrotechnic product preferably includes an assemblage of elongated combustible shreds, these 1000 being flexible shreds of excelsior, each having the described coating *c*. When the shreds are flexed by the action of heat, or otherwise, they cause rupture of the coatings *c*, the latter being frangible, whereby simultaneous combustion of the 105 shreds and of the combustible ingredients of the coatings *c* is permitted, so that during combustion color is emitted simultaneously from the internal and external surfaces of the coatings, the intensity of the emitted color being greater than 110.

would be the case if combustion occurred only on, and progressed only inwardly from the external surfaces of the coatings.

Another advantage of the elongated flexible shreds is found in the fact that when a multiplicity of uncoated shreds, and a suitable quantity of the described semi-fluid paste are assembled in a rotary cement mixer and tumbled, the paste forms the coatings on the shreds, and detachments of the coated shreds are automatically segregated and accumulated by the tumbling operation to form approximately globular masses or balls, each such as that shown by Figure 2, the number of such masses depending on the number of shreds tumbled. These masses may be marketed enclosed in a box.

What is claimed is,

1. A pyrotechnic product composed of an assemblage of elongated combustible shreds independent of each other, each having a coating adhering thereto, each coating including a combustible flame-coloring ingredient, a combustible binding ingredient, and a comminuted refractory combustion-retarding ingredient, the shreds being flexible and the coatings frangible, so that the coatings are rupturable by flexure of the shreds to permit simultaneous combustion of the shreds and of the combustible ingredients of the coatings, so that, during combustion, color is emitted simultaneously from the internal and external surfaces of the coatings.

2. As an article of manufacture, a pyrotechnic product composed of a multiplicity of elements, each including a combustible core and a coating covering and adhering to the core, said coating including a refractory comminuted ingredient, a glow-emitting flame-coloring ingredient, and an adhesive constituting a binding ingredient, said ingredients being intimately mixed, the refractory ingredient retarding the combustion of the binder, the glow emission by the coloring ingredient, and the combustion of the core, when said product is applied to a fireplace fire, so that the flame coloring effect is prolonged, said elements being assembled to form a mass in which the elements adhere to each other, the mass being of suitable size to be deposited on a fireplace fire, and consumed as a unit.

3. That improvement in the method of making a pyrotechnic product which consists in assembling a multiplicity of elongated flexible combustible shreds and a semi-fluid adhesive paste including a combustible flame-coloring ingredient, a combustible binding ingredient and a refractory comminuted combustion-retarding ingredient, tumbling the assembly until the paste forms coatings on the shreds, and detachments of the coated shreds are segregated and assembled to form globular masses, and then solidifying the coatings by drying.

ALTHEA T. BERRY 105

158

110

103

115

153

120

508

125

558

130

606

135

656

140

706

145

751

150

80

85

90

95

100